

May 9, 1961

M. B. DELL ET AL

2,983,665

## UTILIZATION OF LOW-TEMPERATURE TARS

Filed Dec. 23, 1957



INVENTORS  
*Manuel Benjamin Dell &*  
BY *Philip T. Stroup*  
*Peter L. Lester*  
ATTORNEY

# United States Patent Office

2,983,665

Patented May 9, 1961

1

2,983,665

## UTILIZATION OF LOW-TEMPERATURE TARS

Manuel Benjamin Dell, New Kensington, and Philip T. Stroup, Lower Burrel Township, Westmoreland County, Pa., assignors to Aluminum Company of America, Pittsburgh, Pa., a corporation of Pennsylvania

Filed Dec. 23, 1957, Ser. No. 704,575

7 Claims. (Cl. 208—39)

This invention relates to the utilization of tars produced in the low-temperature carbonization of bituminous materials. More particularly, it is directed to a method wherein low-temperature tars, or fractions thereof, are thermally decomposed to high-quality coke suitable as an electrode aggregate and to liquid products which are thermolytically treated to obtain an aromatic pitch suitable as an electrode binder.

Peat, brown coal, lignite, sub-bituminous and bituminous coals are bituminous materials which have been proposed as feedstocks for low-temperature carbonization processes to secure chars or cokes for use as fuel, and tars from which valuable products might be obtained. The present invention is directed to the utilization of such low-temperature tars and to the thermal treatment of fractions thereof to produce aromatic pitch and other valuable materials.

The term "low-temperature carbonization," as used herein, refers to a process for the carbonization of bituminous materials at temperatures lower than about 1300° F. Representative of such a process is that described by V. F. Parry in U.S. Patent 2,773,018 and in "Drying and Carbonizing Fine Coal in Entrained and Fluidized State," Bureau of Mines Report of Investigations 4954, U.S. Department of Interior, dated April 1953.

The term "low-temperature tar," as used herein, refers to tars produced by low-temperature carbonization of peat, brown coal, lignite, sub-bituminous or bituminous coals. Such tars are generally oily, tarry organic masses ranging from viscous liquids to soft semi-solid materials at room temperature and may contain small quantities of char, ash or other inert material, dissolved gases and water.

A typical analysis of low-temperature tar obtained by carbonization of Texas lignite at 946° F. utilizing the Parry Process, supra, is shown in Table 1 below:

TABLE 1

### Analysis of crude tar

|                                                      |        |
|------------------------------------------------------|--------|
| Ash, weight percent                                  | 0.35   |
| Specific gravity, 60°/60° F.                         | 0.9867 |
| Moisture, weight percent                             | 2.9    |
| C-I (quinoline-insolubles), weight percent           | 1.41   |
| Distillation ASTM D20-52, dry basis, weight percent: |        |
| To 170° C.                                           | 2.2    |
| 170-235° C.                                          | 18.4   |
| 235-270° C.                                          | 12.6   |
| 270-300° C.                                          | 12.8   |
| 300° C. to decomposition temperature                 | 31.3   |
| Residue at decomposition temperature                 | 19.7   |
| Loss                                                 | 3.0    |
| Decomposition temperature, ° C.                      | 329    |

2

### Analysis of distillate, vol. percent:

|                                |      |
|--------------------------------|------|
| Tar bases                      | 4.3  |
| Tar acids                      | 23.9 |
| Neutral oil                    | 71.8 |
| Hydrocarbon types <sup>1</sup> |      |
| Saturates                      | 14   |
| Olefins                        | 40   |
| Aromatics                      | 46   |

<sup>1</sup> Method disclosed in article by G. U. Dinneen et al., "Shale Oil Naphthas: Analysis of Small Samples by Silica Gel Adsorption Method," Analytical Chemistry, Vol. 19, p. 992 (1947).

Low-temperature carbonization is generally favored for the production of large quantities of tar as compared to high-temperature processes, thus permitting recovery of considerably greater amounts of tar oils. However, considerable differences exist in the nature of the tars. High-temperature tars are completely aromatic and about 90 percent consists of 3 to 7 ring aromatic compounds with molecular weights up to 400, the remainder consisting of higher molecular weight carbonaceous compounds; in addition, the percentage of phenolic constituents is low, about 5 to 12 percent, but substantially all of these are low-boiling tar acids. Low-temperature tar is only partially aromatic, i.e. about 10-45 percent. It contains relatively large quantities of phenolic constituents, ranging from 20 to 45 percent of the tar; however, these are about evenly distributed in the valuable low-boiling phenolic range and in the higher boiling fraction.

The by-product recovery treatment of such tars may involve a distillation process to recover low-boiling oils from which tar acids are recovered. These phenolic constituents are usually a readily marketable commodity and constitute a definite enhancement to the value of the products obtainable from the process. Tar bases may also be extracted from the distillate, although they are of less commercial significance. Heretofore, the neutral oils remaining after such extraction have been considered generally only as fuel oils because of the high content of sulfur and other heteroatoms. The pitch residue, which constitutes about 25 to 80 percent of the original tar, has generally been considered of poor economic value and used as a fuel or briquetting binder. Much experimental work has been devoted to the development of more valuable uses for this pitch, including the preparation of binders for carbon products.

Binder pitches for carbon products, especially anodes for use in the electrolytic production of aluminum, must meet certain minimum standards. Generally, such anodes must have low resistivity and low reactivity, and it has been found that these properties are obtained when the binder is one of high aromaticity and relatively low quinoline-insolubles content. Pitches obtained by distillation of low-temperature tars fail to meet these criteria, especially with respect to aromaticity.

Aromaticity of binder pitch as measured by the infrared index<sup>1</sup> is considered to be a substantially reliable guide to the suitability of a binder. Analysis of various data on binders when related to the properties of the electrode have indicated that the aromaticity of the binder pitch is one of the most significant factors in producing electrodes having low resistivities and low reactivities. Indicative of this is Table 2 in which properties of various pitches and the carbon anodes produced thereby are listed.

<sup>1</sup> The infrared index of the various pitches indicated herein was determined by a method in which 0.250 gram of pitch is dissolved in 10 ml. of carbon disulfide and allowed to stand for two hours. The infrared spectrum of the supernatant liquid is determined using a cell width of 0.50 mm. in a (Perkin-Elmer Model 112) Spectrometer. After correcting for absorption of the solvent, the infrared index is taken as the ratio of the transmittance at the 3.4 microns aliphatic absorption range divided by the transmittance at the 3.3 microns aromatic absorption range.

TABLE 2  
*Properties of anodes prepared with various binders*

| Binder                                                  | Pitch Properties           |                              |                               |                              |                   | Anode Properties                          |                                          |                                               |
|---------------------------------------------------------|----------------------------|------------------------------|-------------------------------|------------------------------|-------------------|-------------------------------------------|------------------------------------------|-----------------------------------------------|
|                                                         | S.P. <sup>1</sup> ,<br>°C. | C-I, <sup>2</sup><br>Percent | C-II, <sup>3</sup><br>Percent | Coking <sup>4</sup><br>Value | Infrared<br>Index | Baked <sup>5</sup><br>Apparent<br>Density | Resis-<br>tivity <sup>6</sup><br>ohm-in. | Sulfate<br>Reactivity <sup>7</sup><br>Percent |
| Coke-Oven                                               | 109                        | 16.5                         | 33.0                          | 44.1                         | 1.38              | 1.46                                      | 0.0028                                   | 2.4                                           |
| Coke-Oven                                               | 109                        | 7.6                          | 32.0                          |                              | 1.37              | 1.43                                      | 0.0029                                   | 4.7                                           |
| Unknown Foreign                                         | 104                        | 11.5                         | 24.8                          | 35.2                         | 1.08              | 1.41                                      | 0.0030                                   | 5.7                                           |
| Petroleum Oil-Gas                                       | 116                        | 13.3                         | 37.2                          | 42.8                         | 1.01              | 1.41                                      | 0.0028                                   | 7.0                                           |
| Straight Distillation of Bituminous Low-Temperature Tar | 87                         | 0.2                          | 4.6                           | 11.1                         | 0.47              | 1.39                                      | 0.0031                                   | 80.0                                          |
| Straight Distillation of Lignite Low-Temperature Tar    | 111                        | 17.7                         | 28.4                          | 29.3                         | 0.29              | 1.37                                      | 0.0042                                   | 100.0                                         |

<sup>1</sup> Softening point determined by cube-in-air (Barrett method).

<sup>2</sup> Quinoline-insolubles content.

<sup>3</sup> Acetone-insolubles less C-I (quinoline-insolubles).

<sup>4</sup> ASTM D271-48 (paragraph 14c).

<sup>5</sup> The anode is weighed dry, then soaked for 24 hours in water containing few drops of a detergent solution. It is suspended in water and weighed; then it is removed, dried with a towel and weighed while wet. The difference between the weight in water and wet weight is determined and this figure is divided into the dry weight to give the baked apparent density.

<sup>6</sup> A current of known amperage is passed through a cylindrical anode, and a set of probes is used to determine the voltage drop along the longitudinal axis. Resistivity is then calculated by the formula:

$$\rho = \frac{(E)(A)}{(I)(D)}$$

Where

$\rho$  = resistivity in ohm-inches

E = average voltage drop across probes

A = cross-sectional area of sample (square inches)

I = current passed through samples (amperes)

D = distance between probes (inches)

<sup>7</sup> Sulfate reactivity is the loss in weight of a carbon specimen, 1 inch in diameter by  $\frac{1}{2}$  inch, when immersed in molten sodium sulfate at  $940^{\circ}$  C. It is considered an excellent measure of the reactivity of an anode in a bath for the production of aluminum by the Hall process.

It has now been found that low-temperature tars, or fractions thereof, may be converted from substantially non-aromatic material to an aromatic tar from which a binder pitch suitable for carbon electrodes may be obtained by distillation. This conversion is effected by thermally cracking the tar or tar fraction at a temperature of  $700^{\circ}$  C. to  $900^{\circ}$  C. and at atmospheric or low superatmospheric pressure. The aromaticity of the binder pitch is indicated by the infrared index, as hereinbefore described. Table Three illustrates the conversion effected and the quality of the binder pitch obtained by such thermal conversion of a lignite tar fraction.

the high-boiling tar acids in low-temperature tars to the more valuable low-boiling tar acids.

Further objects and advantages of the present invention will be evident from the attached drawing and following detailed description.

It has been found that low-temperature tars may be substantially completely utilized by a method in which the tar, or a fraction thereof, is thermally decomposed into a high-quality coke, gas and condensable oils. The condensable oils, or a fraction thereof, are then thermally cracked at a temperature between  $700^{\circ}$  C. and  $900^{\circ}$  C. and at a pressure between atmospheric and low superatmospheric, the products being gas, liquid products in-

TABLE 3  
*Properties of anodes prepared with various binder pitches*

| Pitch                                      | Pitch Properties |                   | Anode Properties             |                               |                                                                  |
|--------------------------------------------|------------------|-------------------|------------------------------|-------------------------------|------------------------------------------------------------------|
|                                            | S.P.,<br>°C.     | Infrared<br>Index | Baked<br>Apparent<br>Density | Resis-<br>tivity,<br>ohms-in. | Sulfate<br>Reactivity,<br>Percent<br>Loss at<br>$960^{\circ}$ C. |
| Lignite by Straight Distillation           | 102              | 0.15              | 1.43                         | 0.0030                        | 64                                                               |
| 100 Lignite Thermolytic Pitch <sup>1</sup> | 117              | 1.01              | 1.49                         | 0.0026                        | 40                                                               |
| 50% Lignite Thermolytic Pitch              |                  |                   | 1.47                         | 0.0027                        | 28                                                               |
| 50% Coke-Oven Pitch                        |                  |                   | 1.48                         | 0.0027                        | 41                                                               |
| Coke-Oven Pitch                            | 107              | 1.32              |                              |                               |                                                                  |

<sup>1</sup> Lignite thermolytic pitch was obtained by thermally cracking lignite low-temperature tar residue by a cyclic regenerative process at an average temperature of  $779^{\circ}$  C. and at 1.10 atmospheres pressure.

It is an object of this invention to provide a method for the substantially complete utilization of low-temperature tars.

Another object is to provide a method for the treatment of low-temperature tars whereby an aromatic pitch suitable as an electrode binder is obtained.

It is also an object to provide a method wherein low-temperature tars are utilized to produce high-quality coke suitable as an aggregate for carbon electrodes and other valuable products.

A further object is to provide a method for cracking

including a thermolytic tar, and carbon or coke. The thermolytic tar is then distilled to an aromatic pitch having the desired physical properties and an aromatic oil.

Preferably, the whole or crude low-temperature tar is initially distilled to recover phenolic oil prior to the thermal decomposition; it is also desirable to fractionate the condensable oils from the thermal decomposition so as to recover a second phenolic oil, the balance of the condensable oils, or middle oil, being used as the feedstock for the thermal cracking. These phenolic oils are desirably processed to recover tar acids and tar bases,

leaving a neutral oil which also may be thermally cracked, either separately or in admixture with the middle oil. The aromatic oil from the pitch distillation is also desirably fractionated into phenolic and middle oils, and the tar acids and tar bases may be removed also from this phenolic oil. Similarly, the various oils may be caustic-washed only to remove the tar acids alone.

More particularly, the thermal decomposition is effected at a temperature between 375° C. and 475° C. and a pressure between atmospheric and 100 pounds per square inch.

A cyclic regenerative process has been found essential to the practicable thermal cracking of low-temperature tars because of the tendency of this material to form large quantities of carbon at cracking conditions. This carbon deposition will choke a continuous reactor, prevent maintenance of uniform cracking conditions and contaminate the product stream, especially the tar from which the aromatic pitch is derived.

The terms "low-temperature tar feedstock" or "tar feedstock," as used herein, refer to crude or whole low-temperature tars, or to fractions thereof, such as the residues upon topping, or distillates.

The term "phenolic oil," as used herein, refers to a tar distillate relatively rich in valuable phenolic constituents, such as phenol, cresols, xylenols, and ethyl phenols. It is preferred to use about 235° C. as the end point for this distillate although variations may be made dependent upon the compounds desired in this fraction.

The term "middle oil," as used herein, refers to a tar distillate boiling above the phenolic oil range.

The term "tar distillate," as used herein, refers to any distillate from low-temperature tars or from tars formed in the thermal treatment of low-temperature tar, and may encompass phenolic oil, or middle oil, or both.

The apparatus for effecting the thermal decomposition may be of any type capable of affording the conditions of temperature and pressure herein described. A delayed coker is preferably employed, although other types, such as a pot still, may be satisfactorily utilized.

Generally, the temperature of the thermal decomposition is between 375° C. and 475° C. and preferably between 380° C. and 420° C. The pressures employed may vary between atmospheric and 100 pounds per square inch. The pressure selected will depend largely upon the character of the feedstock, but about 40 to 60 pounds per square inch is preferable.

A portion of the condensable oils such as the middle oil fraction may be recycled and mixed with the tar feedstock prior to the preheater. By so doing, especially in the case of topped tar, the feedstock is more easily transported and premature coking is substantially eliminated. Generally, this recycle ratio may be between 0.3 and 3.0 times the feedstock, and preferably between 0.5 and 1.5.

The ash content of the coke produced by the process will be dependent upon that of the feedstock. Particularly for the production of anodes for electrolytic reduction cells, it is desirable that the coke contain as little ash as possible and generally less than about 0.8 percent. Thus when employing low-temperature tars which usually contain considerable quantities of ash, it has been found desirable to reduce the solids contained in the feed tar prior to the thermal decomposition. For this purpose, several methods may be employed such as, for example, those disclosed in U.S. Patents 2,631,982 to Donegan and 2,774,716 to Kulik.

The term "cyclic regenerative process," as used herein, refers to a semi-continuous process for thermolytic cracking of tar feedstocks wherein a cycle of operation for the cracking apparatus includes a period in which the carbon deposits within the apparatus are removed by combustion. Such a cycle generally includes a heating period in which the apparatus is heated to cracking

temperatures, a cracking or make period in which thermolysis of feed takes place, and a blast period in which the carbon deposits are burned, the last of which may be in conjunction with the heating period. The heat developed by combustion of the carbon deposits is transferred substantially to heat-storing surfaces which subsequently impart heat to the feed and to the carrier gas if such is used. Subsequent to the cracking period, heat retained by these heat-storing surfaces is transferred to the oxidizing gas which is introduced to burn the carbon deposits. This type of process is extensively used to produce fuel gas from petroleum oils and the apparatus employed may conveniently be of the type known as the "oil-gas set."

The term "oil-gas set," as used herein, refers to any cyclic, regenerative thermal cracking apparatus, and may be of the type illustrated and described in U.S. Patent 2,721,123 to E. S. Pettyjohn et al. and U.S. Patent 2,580,766 to E. L. Hall. The essential features of this apparatus are that it be cyclic, regenerative, capable of providing temperatures of about 700° C. to 1100° C., and afford suitable collecting means for the tar and other products.

Generally, an apparatus for cyclic regenerative cracking comprises one or more generating vessels or zones in communication with two or more regenerator (superheater) vessels or zones, the several vessels or zones being provided with heat-storing surfaces, preferably of a highly heat-conductive material such as carborundum or silicon carbide.

In the operation of the apparatus, there is a blast period in which the generator vessel or zone is heated to cracking temperatures by combustion of carbon previously deposited on the heat-storing surfaces and/or fuel oil or gas. The combustion products are usually discharged through one of the regenerator vessels or zones in order to heat the surfaces therein. In the make or cracking period, a diluent or carrier gas is usually provided and is introduced into the apparatus (generally through the heated regenerator) wherein it is heated by contact with the heat-storing surfaces. The feedstock is sprayed into the generator, usually with the aid of an atomizing diluent or carrier gas, wherein it admixes with the heated carrier gas and wherein it is initially cracked. These initial products are conducted through the second regenerator wherein further cracking may take place prior to discharge. In some apparatus cracking is completed in the generators and the cracking products discharged without passing through the regenerators. Suitable means are provided to collect both the process gas and the condensable products such as tar and light oil, either separately or together.

Referring now to the attached drawing, diagrammatically illustrated is a process embodying the present invention. A low-temperature tar 2 is preferably topped in still 4 to recover a phenolic oil 6, leaving a residue 8, which is then thermally decomposed in retort 10 to yield green coke 12, process gas 14 and condensable oils or condensate 16.

In column 18 the condensate 16 is fractionated into phenolic oil 20 and middle oil 22, a part of which is desirably recycled and admixed with the residue 8 prior to thermal decomposition. The middle oil 22 is then thermolytically cracked in retort 24, preferably in the presence of a carrier gas 26, and the products withdrawn are process gas 28, which is right in olefins, and liquid products including a thermolytic tar 30 (a light oil fraction may be collected separately if so desired). After separation of water, the thermolytic tar 30 is distilled or topped in still 32 to a highly aromatic pitch 34 suitable as a carbon electrode binder, and an aromatic oil 36 which may be fractionated in the column 38 to middle oil 40 and phenolic oil 42 from which considerable

quantities of valuable low-boiling tar acids, tar bases and other chemicals may be extracted.

The phenolic oil 6 is desirably subjected to a conventional treatment 44 to recover the tar bases 46, which treatment may be of the type utilizing dilute acid, and to a second treatment 48 to remove the tar acids 50, such as by the conventional methods of washing with caustic solution or solvents, leaving a neutral oil 52. The phenolic oil 20 contains considerable quantities of low-boiling tar acids and tar bases which have been formed by the higher-boiling constituents during the thermal decomposition in retort 10, and is desirably processed in treatment plants such as 44 and 48.

The thermolytic phenolic oil 42 from the column 38 is also desirably processed to recover the low-boiling phenolic compounds and nitrogen-bases; the plants 44 and 48 may be conveniently employed although it is preferable that this material be processed separately to maintain the identity of the neutral oil resulting from treatment of this highly aromatic oil.

The process gas 28 which consists largely of methane, ethane, ethylene and hydrogen may be treated to extract the olefins and recycled as the carrier gas 26 for the thermolytic cracking, or it may be used as a heating gas.

The green coke 12 is desirably calcined in retort 54 at a temperature above 1000° C. to obtain a high-quality aggregate 56 suitable for carbon electrodes.

The average effective temperature in the thermal cracking apparatus is generally maintained between about 700° C. and 900° C., and preferably about 760° C. to 820° C. Higher temperatures are found to favor the formation of deposited carbon over the formation of liquid products, and to increase the C-I (quinoline-insoluble) content of the tar, whereas lower temperatures do not generally provide sufficient cracking to form aromatic tars. The conditions of temperature may be varied, of course, if the residence time is varied; i.e., higher temperatures may be compensated by lower residence times, and vice versa. When the pressure within the apparatus is varied within the usual range, namely, from atmospheric to about 25 pounds per square inch, the throughput rate may be adjusted to maintain constant residence time. Higher pressures, up to about 50 p.s.i., may be employed; however, there is little increase in tar yield because of increased carbon formation due to increased tendency to the occurrence of stagnant conditions. The residence times normally employed at atmospheric or low super-atmospheric pressure are from 1 to 10 seconds, and preferably about 2 to 5 seconds; shorter times are not sufficient to produce the degree of cracking desired unless higher temperatures are also employed, whereas longer residence times produce excessive cracking unless reduced temperatures are employed. For an average cracking temperature of 760° C. to 820° C. at atmospheric or low super-atmospheric pressure, a residence time of 2½ to 4 seconds has been found most effective.

The operating cycle (or half-cycle if a symmetrical unit is employed) may be between 1 and 20 minutes and is usually about 3 to 6 minutes. The length of the cycle is, of course, determined by the physical capabilities of the unit and the degree of variation in conditions which may be tolerated. However, for a unit of the type described in the Pettyjohn patent, supra, a cycle (half-cycle) on the order of about 4 minutes is preferred.

In the operation of a cyclic regenerative unit, a carrier gas has been found desirable to assist in the transportation of the cracking products as well as to function as a heat-carrier. However, the cracking products themselves may be used as the motivating agent, although much less effective. Various carrier gases may be employed, such as steam, inert gas, hydrogen-rich gas, or the like; an amount of steam up to about 2 pounds per gallon of feedstock is usually employed in such units.

In accordance with this invention, lignite low-temperature tar, substantially as described in Table 1, was distilled

to recover phenolic oil. Data on this distillation are presented in Table 4 below:

TABLE 4

*Initial distillation of crude lignite tar*

|                                         |      |
|-----------------------------------------|------|
| Max. temp., ° C.                        | 235  |
| Products, wt. percent:                  |      |
| Phenolic oil                            | 27.8 |
| Residue                                 | 72.2 |
| Residue properties:                     |      |
| Specific gravity, 60°/60° F.            | 1.07 |
| C-I (quinoline-insolubles), wt. percent | 0.42 |
| Ash, wt. percent                        | 0.92 |
| Moisture, wt. percent                   | 1.3  |
| Sulfur, wt. percent                     | 0.99 |
| Phenolic oil composition, vol. percent: |      |
| Tar bases                               | 3.8  |
| Tar acids                               | 22.6 |
| Neutral oil                             | 73.6 |
| Hydrocarbon types, vol. percent—        |      |
| Saturates                               | 7    |
| Olefins                                 | 44   |
| Aromatics                               | 47   |

Lignite low-temperature tar residue from phenolic oil distillation, substantially as described in Table 4, was thermally decomposed in a delayed coker to obtain process gas, green coke and condensate as shown in Tables Five and Six below.

TABLE 5

*Thermal decomposition*

|                                                       |      |
|-------------------------------------------------------|------|
| Conditions:                                           |      |
| Temp., ° C.                                           | 425  |
| Pressure, p.s.i.g.                                    | 50   |
| Product Yields:                                       |      |
| Coke, green, wt. percent of feed                      | 26.1 |
| Gas, cu. ft. per lb. of feed                          | 1.18 |
| Condensate, wt. percent of feed                       | 62.8 |
| Phenolic oil (to 235° C.), vol. percent of condensate | 32.0 |
| Middle oil (over 235° C.), vol. percent of condensate | 68.0 |

TABLE 6

*Product analysis*

|                                       |      |
|---------------------------------------|------|
| Gas, mol percent:                     |      |
| H <sub>2</sub>                        | 4.9  |
| CH <sub>4</sub>                       | 46.3 |
| C <sub>2</sub> H <sub>6</sub>         | 15.4 |
| C <sub>3</sub> H <sub>8</sub>         | 7.7  |
| C <sub>2</sub> H <sub>4</sub>         | 2.5  |
| C <sub>3</sub> H <sub>6</sub>         | 3.8  |
| CO                                    | 5.6  |
| CO <sub>2</sub>                       | 5.7  |
| Condensate composition, vol. percent: |      |
| Tar bases                             | 2.6  |
| Tar acids                             | 18.7 |
| Neutral oil                           | 78.7 |
| Hydrocarbon types, vol. percent—      |      |
| Saturates                             | 25   |
| Aromatics                             | 40   |
| Olefins                               | 35   |
| Distillation ASTM D-86:               |      |
| Initial, ° C.                         | 51   |
| 10 ml.                                | 167  |
| 20 ml.                                | 207  |
| 30 ml.                                | 231  |
| 40 ml.                                | 251  |
| 50 ml.                                | 260  |
| 60 ml.                                | 284  |
| 70 ml.                                | 331  |
| 85.8 ml.                              | 337  |
| Decomposition, ° C.                   | 337  |
| Residue, percent                      | 10.8 |

The condensate was fractionated into phenolic oil and

middle oil. The middle oil was then thermally cracked to yield thermolytic tar, light oil and a process gas; the carbon or coke formed by the cracking was substantially deposited within the apparatus and subsequently removed by combustion. Data on this thermolysis are presented in Table 7.

TABLE 7

*Thermolytic cracking*

## Operating conditions:

|                              |       |
|------------------------------|-------|
| Carrier gas, type            | Steam |
| Carrier gas, s.c.f./gal.     | 22.8  |
| Total pressure, atm.         | 1.0   |
| Cracking temp., average, °C. | 7.66  |
| Residence time, sec.         | 3.4   |

## Product yields:

|                                         |      |
|-----------------------------------------|------|
| Total gas, s.c.f./gal.                  | 46.7 |
| Thermolytic tar, percent by wt. of feed | 63.7 |
| Light oil, percent by wt. of feed       | 1.8  |

## Product gas composition, mol. percent:

|                               |      |
|-------------------------------|------|
| H <sub>2</sub>                | 15.1 |
| CH <sub>4</sub>               | 39.9 |
| C <sub>2</sub> H <sub>6</sub> | 5.1  |
| C <sub>3</sub> H <sub>4</sub> | 20.7 |
| C <sub>3</sub> H <sub>6</sub> | 7.2  |
| CO                            | 8.9  |
| Others                        | 3.1  |
| Heating value, B.t.u./s.c.f.  | 1145 |

## Thermolytic tar properties:

|                                         |       |
|-----------------------------------------|-------|
| Specific gravity, 60°/60° F.            | 1.110 |
| C-I (quinoline-insolubles), wt. percent | 5.0   |

The thermolytic tar described in Table 7 was topped

## Properties of pitch:

|                                            |       |
|--------------------------------------------|-------|
| Softening point, °C.                       | 107   |
| Specific gravity, 60°/60° F.               | 1.263 |
| Ash, percent by wt.                        | 0.30  |
| C-I (quinoline-insolubles), percent by wt. | 9.9   |
| Infrared index                             | 1.01  |
| Sulfur, percent by wt.                     | 0.97  |

## Analysis of aromatic oil:

|                               |      |
|-------------------------------|------|
| Sulfonation index (ASTM D872) | 0.9  |
| Tar acids, vol. percent       | 14.1 |
| Tar bases, vol. percent       | 5.5  |
| Neutral oil, vol. percent     | 80.4 |

As is evident from the infrared index, the low-temperature tar has been converted to an aromatic pitch of relatively low C-I (quinoline-insolubles) content. Thermolytic pitches having these properties are suitable binders for carbon electrodes and produce anodes of low resistivities, as shown in Table 3. Further, the binder of the present invention may be used alone or in combination with other pitches such as, for example, coke-oven pitch as shown in Table 3.

The green coke from the thermal decomposition was calcinated at a temperature of about 1200° C. for 20 hours. The properties of the calcined material and of anodes prepared therewith were determined, comparison determinations being made for commercially available petroleum coke. As evidenced by the data in Table 9, the coke made in accordance with the present invention produces electrodes of greatly improved resistivity; the baked apparent density is superior and the sulfate reactivity is in the acceptable range and substantially equivalent to that of petroleum coke.

TABLE 9

| Coke      | Coke                         |                  |                                    | Anode <sup>1</sup>     |                       |                                 |
|-----------|------------------------------|------------------|------------------------------------|------------------------|-----------------------|---------------------------------|
|           | Volatile Matter, Wt. percent | Ash, wt. percent | Resistivity, <sup>2</sup> ohms-in. | Baked Apparent Density | Resistivity, ohms-in. | Sulfate Reactivity <sup>3</sup> |
| Petroleum | 0.14                         | 0.45             | 0.0549                             | 1.50                   | .0026                 | 59                              |
| Lignite   | 0.00                         | 4.14             | 0.0484                             | 1.52                   | .0022                 | 69                              |

<sup>1</sup> Anodes made with 110° C. softening point coke-oven pitch.

<sup>2</sup> Great Lakes Carbon Co. Procedure No. C-12A.

<sup>3</sup> Sulfate reactivity determined at 960° C.

in a pitch still to obtain an aromatic binder pitch having a softening point of about 110° C. and a highly aromatic oil distillate which contained low-boiling phenolic constituents. The properties of the pitch and the aromatic oil are shown in Table 8.

TABLE 8

*Distillation of thermolytic tar*

## Distillation, wt. percent:

|              |      |
|--------------|------|
| 100°-120° C. | 0.5  |
| 120°-140°    | 0.9  |
| 140°-160°    | 1.5  |
| 160°-180°    | 2.3  |
| 180°-200°    | 3.7  |
| 200°-230°    | 5.6  |
| 230°-300°    | 23.5 |
| 300°-350°    | 20.4 |
| Pitch yield  | 41.4 |

## Product yields, percent by wt.:

|              |      |
|--------------|------|
| Aromatic oil | 58.6 |
| Pitch        | 41.4 |

The use of a hydrogen-rich carrier gas has been found desirable in the production of an aromatic pitch. The process gas, which consists largely of methane (25 to 35 percent) and hydrogen (15 to 20 percent), may be stripped of the olefins and used to decrease materially the C-I (quinoline-insolubles) or carbon content of the thermolytic tar and resultant binder pitch. Illustrative of this effect are the analyses shown in Table 10, wherein the results from using hydrogen and methane are compared to those from using steam.

TABLE 10

*Properties of binder pitch*

| Carrier Gas                             | Steam | Methane | Hydrogen |
|-----------------------------------------|-------|---------|----------|
| Softening point, °C.                    | 105   | 115     | 110      |
| Specific gravity, 60°/60° F.            | 1.294 | 1.296   | 1.289    |
| C-I (quinoline-insolubles), wt. percent | 23.3  | 17.9    | 12.1     |
| Infrared index                          | 1.00  | 1.13    | 1.09     |
| Sulfur, wt. percent                     | 0.71  | 0.71    | 0.78     |

The aromatic neutral oil remaining after tar acid and tar base extraction of the phenolic oil from the thermolytic tar distillation has been found to contain large percentages of naphthalenic compounds, generally about 70 percent. It is thus desirable that this oil be processed separately from other streams to preserve its identity and to facilitate recovery of these constituents.

Having thus described the invention, we claim:

1. In the production of high-quality coke and aromatic pitch from low-temperature tars, the method comprising thermally decomposing a low-temperature tar feedstock at a temperature between 375 and 475° C. and a pressure between atmospheric and 100 pounds per square inch to obtain coke, gas and condensable oils; thermally cracking at least part of said condensable oils at a temperature between 700° and 900° C., at a pressure between atmospheric and low superatmospheric and at a residence time of 1 to 10 seconds to yield gaseous and liquid products including a thermolytic tar; and distilling said thermolytic tar to an aromatic pitch and an aromatic oil.

2. The method in accordance with claim 1 wherein the low-temperature tar feedstock is whole low-temperature tar.

3. The method in accordance with claim 1 wherein the low-temperature tar feedstock is the residue from distilling whole low-temperature tar to recover phenolic oil.

4. In the production of coke and aromatic pitch from low-temperature tars, the method comprising distilling low-temperature tar to recover phenolic oil; thermally decomposing the residue from said phenolic oil distillation at a temperature between 375° C. and 475° C. and a pressure between atmospheric and 100 pounds per square inch, thereby yielding coke, gas and condensable oils containing phenolic constituents; thermally cracking at least part of said condensable oils by a cyclic regenerative process at a temperature between 700° C. and 900° C., at a pressure between atmospheric and low super-

atmospheric and at a residence time of 1 to 10 seconds to obtain gaseous and liquid products including a thermolytic tar; distilling said thermolytic tar to an aromatic pitch; recovering from said second-mentioned distillation an aromatic oil containing phenolic constituents; and extracting phenolic constituents from said phenolic oil, from at least part of said condensable oils and from at least part of said aromatic oil.

5. The method in accordance with claim 4 wherein condensable oils are recycled and admixed with said residue in an amount between 0.3 and 3.0 to 1.0 prior to the said thermal decomposition step.

6. The method in accordance with claim 4 wherein said condensable oils are thermally cracked in the presence of a hydrogen-rich carrier gas.

7. The method in accordance with claim 6 wherein at least part of said gaseous products from the said thermolytic cracking are recycled to provide said hydrogen-rich carrier gas.

20

References Cited in the file of this patent

UNITED STATES PATENTS

|           |                 |               |
|-----------|-----------------|---------------|
| 2,039,835 | Petersen et al. | May 5, 1936   |
| 2,098,033 | Fischer         | Nov. 2, 1937  |
| 2,658,857 | Roediger        | Nov. 10, 1953 |
| 2,772,219 | Dunkel et al.   | Nov. 27, 1956 |
| 2,847,357 | Moser           | Aug. 12, 1958 |

FOREIGN PATENTS

30 30 457,971 Great Britain Dec. 7, 1936

OTHER REFERENCES

Egloff et al.: Cracking of Low Temperature Coal Tar by the Dubbs Process, published by Universal Oil Products Co. (1926), pp. 1 to 11.

Dunstan: Internal Conference on Bituminous Coal, November 1928, pp. 210 to 231, volume 1.